

## UNITED STATES PATENT OFFICE.

JOHN P. DELZEIT, OF TAMAQUA, PENNSYLVANIA, ASSIGNOR TO THE LEHIGH COAL AND NAVIGATION COMPANY, OF PHILADELPHIA, PENNSYLVANIA, A CORPORATION OF PENNSYLVANIA.

## BRIQUETTE AND PROCESS OF MAKING THE SAME.

No Drawing.

Application filed December 4, 1925. Serial No. 73,258.

The invention relates more particularly to fuel briquettes utilizing sulfite liquor, molasses, molasses residue, desugared molasses or similar substances as one ingredient of their binder. Briquettes made with binders of the above nature have usually proved to be weak in their weather resisting qualities, and their manufacture has required heat treatment over a comparatively long period. 10 The present invention aims to improve briquettes of the above nature, both as to their weather resisting and other qualities, and as to their process of manufacture. One important object is to shorten the time 15 of heat treatment necessary to produce a satisfactory briquette.

Further objects and advantages of the invention will be in part obvious and in part specifically pointed out in the description 20 hereinafter contained, wherein a preferred embodiment of the invention is disclosed; such embodiment, however, is to be considered as merely illustrative of its principles.

I have found that the binding qualities 25 of such substances as sulfite liquor, molasses, and similar organic pitchy compounds obtained in the alcohol and sugar industries, are much improved by adding sulfur, or sulfur containing salts or compounds thereto, particularly in that a satisfactorily weather resistant briquette may be produced with such a binder, by a heat treatment lasting for only about one half hour or even somewhat less, whereas 30 briquettes having binders of sulfite liquor or similar substances have heretofore been unsatisfactory in their weather resisting qualities, even when subjected to heat treatment for a period of two or three hours. 40 The reduction in time of heat treatment results in a considerable decrease in expense of production, and my briquette is also superior from the standpoint of strength.

To prevent disintegration of the briquette 45 by undue burning of the sulfur during heat treatment in an oxidizing atmosphere, I add a certain amount of sulfuric acid to the binder. The sulfuric acid acts during the heat treatment to extinguish quickly any flames which may be produced, and such burning as does take place, strikes inwardly, causing rapid penetration of heat to the center of the briquette and assisting carbonization.

To give a specific example of one mode of carrying out the invention, the binder may consist of the following parts by weight: 1 part of crude powdered sulfur, 3½ parts commercial sulfuric acid, 78 parts sulfite liquor (standard concentrated). Water to 60 make up 100 parts. The ingredients of the binder may be mixed cold in any suitable mixing apparatus, the proportions above given not being at all critical.

Anthracite fines, or other coal desired to 65 be employed, will then be mixed with the binder and formed into briquettes in the usual manner.

The heat treatment of the briquettes may be carried out by means of any suitable 70 oven or furnace, in which the briquettes are raised to a temperature somewhat under 700° F. for a period long enough to make them sufficiently weather resistant. Usually a period of about one half hour will be sufficient. I prefer to employ a long oven, 75 through which the briquettes are carried by a suitable conveying apparatus, so as to raise their temperature gradually up to about 600-650° F. If raised above 700° F., 80 the binding powers of the sulfite liquor become impaired, and it is therefore not desirable to heat the briquettes above that point. The briquettes may then be quenched 85 in any suitable manner.

While a specific embodiment of the invention has been disclosed, it will be obvious 90 that many changes may be made therein without departing from its principles as set forth in the following claims.

I claim:—

1. A fuel briquette, comprising fine coal and a binder having sulfite liquor or the like and a relatively small percentage of sulfur in addition thereto which has been 95 subjected to a carbonizing heat treatment at about 600-700° F.

2. A fuel briquette, comprising fine coal and a binder having sulfite liquor or the like in combination with sulfuric acid and a 100 small percentage of sulfur in addition thereto, which has been subjected to a carbonizing heat treatment at about 600-700° F.

3. The process of making fuel briquettes, which comprises mixing fine coal with a 105 binder having sulfite liquor or the like and a relatively small percentage of sulfur in addition thereto, forming briquettes there-

of, and subjecting the briquettes to a heat treatment at about 600-700° F., for about one-half hour.

4. The process of making fuel briquettes, which comprises mixing fine coal with a binder having sulfite liquor or the like in combination with sulfuric acid and a relatively small percentage of sulfur in addition thereto, forming briquettes thereof, and subjecting the briquettes to a heat treatment at about 600-700° F. for about one-half hour.

5. The process of making fuel briquettes, which comprises mixing fine coal with a binder having sulfite liquor or the like and a relatively small percentage of sulfur in addition thereto, forming briquettes there-

of, and subjecting the briquettes to a low temperature carbonizing heat treatment to render them weather resistant.

20

6. The process of making fuel briquettes, which comprises mixing fine coal with a binder having sulfite liquor or the like in combination with sulfuric acid and a relatively small percentage of sulfur in addition thereto, forming briquettes thereof, and subjecting the briquettes to a low temperature carbonizing heat treatment to render them weather resistant.

25

In testimony that I claim the foregoing, I have hereunto set my hand this 23rd day of November, 1925.

JOHN P. DELZEIT.